

# UNITED STATES PATENT OFFICE.

CHARLES J. THATCHER, OF NEW YORK, N. Y.

## PHOTOGRAPHIC DEVELOPER.

1,158,011.

Specification of Letters Patent.

Patented Oct. 26, 1915.

No Drawing.

Application filed March 22, 1915. Serial No. 16,286.

*To all whom it may concern:*

Be it known that I, CHARLES J. THATCHER, a citizen of the United States, and a resident of New York city, in the county of New York and State of New York, have invented 5 certain new and useful Improvements in Photographic Developers, of which the following is a specification.

This invention relates to improvements in 10 the use of photographic developers.

The object of the invention is to so regulate the action of a photographic developer as to provide a satisfactory substitute for rapid and expensive developers like "metol" 15 (mono-methyl-paramidophenol sulfate); and it has for its further object to effect such regulation of photographic development without producing undesirable or inferior results.

At the present time the organic compound, 20 monomethyl paramidophenol sulfate, usually called "metol", is perhaps the most rapid and at the same time most expensive photographic developer in general use. In 25 commercial photography, at least, it has hitherto not been possible to substitute other cheaper developers for the specified compound, principally because of the lesser speed of development of such other develop-

30 ers. Where large numbers of negatives or positives have to be developed each day, as in the production of moving picture films, it is important that the development should be as rapid as possible. The extreme rapid- 35 ity of the reducing action of monomethyl paramidophenol sulfate upon silver salts, accounts, in a large degree, for its exclusive use—despite its high cost—in combination with hydroquinone, in commercial photog- 40 raphy. I have found that other cheaper de- 45 velopers, paramidophenol sulfate, for ex- ample, may be satisfactorily used, either alone or mixed with hydroquinone for ex- ample, and produce as rapid or more rapid 50 development of the latent image, provided the proper conditions, which I herein dis- close, are employed. In the development of moving picture films, for example, paramido- phenol sulfate may, by my invention, now be substituted for the monomethyl deriva- 55 tive thereof, and produce the same speed, color, density, contrast, etc. with the same formula, by the improvement which I will hereinafter describe.

In the development of moving picture

films, the developing solutions have been made by dissolving in water, metol, hydroquinone, alkali sulfites and carbonates and potassium bromid. Developers containing these constituents have been used for the 60 development of moving picture films since the early days of the art. Such a developing solution requires, for the complete development of a normally printed positive, from two to five minutes. If paramidophenol sulfate is substituted for the monomethyl derivative thereof, using the other ingredients, the development of the same positive requires twice as long. Attempts which have been made to substitute paramidophenol sulfate or hydrochlorid in place of metol have failed and have been abandoned because of the longer time required for the development of the plates or films. I have succeeded in overcoming this difficulty attending the 65 use of paramidophenol and similar developing compounds, by adding a relatively small amount of sodium or potassium hydrate to the developing solution as ordinarily prepared and used.

In the development of moving picture films, for example, I may use the following formula for mixing up the developing solution, as a representative formula.

|                        |     |        |
|------------------------|-----|--------|
| Water                  | 800 | parts. |
| Paramidophenol sulfate | .5  | "      |
| Hydroquinone           | 2   | "      |
| Sodium sulfite         | 20  | "      |
| Sodium carbonate       | 14  | "      |
| Potassium bromid       | .5  | "      |
| Sodium hydrate         | 1   | "      |

The use of 1 part of sodium hydrate in a developing solution containing these constituents and proportions, is, I find, sufficient 95 to regulate the development so that substantially the same results are obtained and in substantially the same time as with a metol-hydroquinone developer of the same composition, but without the sodium hydrate. I 100 give these proportions only by way of example. The proportions may be varied and in some instances it may be necessary to use a larger proportion of sodium hydrate, for example, 2 parts thereof. An equal weight of paramidophenol sulfate may be similarly substituted for the metol in any developing solution formula by adding a sufficient quantity of sodium hydrate to give substantially 105 the same rapidity of development as does 110

the metol developing solution. Generally the proportion of sodium hydrate necessary will be between 1/10 and 1/30 of the amount of sodium carbonate in the developer. As 5 compared to the quantity of paramidophenol sulfate the sodium hydrate may be one to four times as much. It will be understood that to produce this surprising increase in speed of development, by the addition of 10 such a small proportion of sodium hydrate, it is unnecessary to otherwise change the formula in use, although this may be done if desired. The films so produced, moreover, are generally superior as regards color, brilliancy, detail, etc.

Developers, such as a solution of paramidophenol, have been made and used heretofore with sodium hydrate or other caustic alkalis in place of sodium carbonate. An 20 example of such a developer now in use is "rodinal." But for commercial photography, where a large quantity of developing solution is made up at one time and used continuously for a number of days until 25 exhausted, it has been found impossible to economically and satisfactorily use a developing solution of this nature, containing, in addition to the other usual ingredients, a caustic alkaline solution of paramidophenol 30 or of the same and hydroquinone. In the first place sufficient amount of sodium hydrate caused a rapid and unpermissible deterioration of the developing solution by oxidation. Moreover, a solution 35 containing such a quantity of sodium hydrate (without sodium carbonate) caused frilling of the gelatin or partly dissolved it, or produced a mottled effect which became noticeable when the image 40 was projected upon a screen. But by mixing up the developing solution with both the hydrate and the carbonate of sodium or of potassium, and in suitable proportions as previously specified, instead of either the hydrate or carbonate alone, I am able to avoid 45 the disadvantageous effects attending the use of the hydrate alone, and am able to increase, to the necessary degree, the speed of development over that which is obtainable 50 with carbonate alone.

I believe that the explanation of the effect herein disclosed, viz: that a stable, rapid developing solution may be produced by the use of a relatively small proportion of sodium hydrate with the carbonate, is found in the following reaction, which occurs when alkaline carbonates are dissolved in water. Neglecting the sodium anions and considering only the cathions, this reaction is:



This is a reversible reaction and an equilibrium, is constantly maintained between the concentration of the various components 65 of the system. When the hydroxyl—(OH')

concentration is increased, as I do by adding a small amount of sodium hydrate, the reaction proceeds from right to left, partially reducing the concentration of the OH and of the  $\text{HCO}_3$  ions, and correspondingly increasing the concentration of the  $\text{CO}_3$  ion and of water until the equilibrium is restored. The concentration of hydroxyl ions in the solution, at any time, therefore, is not as great as that due to the sodium hydrate 75 alone nor to the sum of this concentration and that due to the sodium carbonate, so that oxidation and deterioration, which varies directly as the hydroxyl concentration, is much slower than in a sodium hydrate solution alone. On the other hand, as the hydroxyl ion concentration tends to decrease during the use of the developing solution, it is restored by the reaction proceeding from left to right to maintain the 80 equilibrium.

It will be understood that my invention may be used for the production of stable, rapidly developing solutions of other developing compounds than paramidophenol sulfate, or 90 of mixtures thereof with hydroquinone, and that suitable changes in the ingredients and proportions hitherto specified may be made by those skilled in the art without departing from the scope of my invention. 95

I claim:

1. The process of rapidly developing the latent image of an exposed, sensitized photographic surface which consists in subjecting the exposed sensitized surface to the 100 action of a solution containing hydroquinone and a relatively smaller proportion of paramidophenol sulfate; an alkali sulfite; an alkali carbonate, and a relatively small proportion of sodium hydrate. 105

2. The process of rapidly developing the latent image of an exposed sensitized photographic surface, which consists in subjecting the exposed sensitized surface to the action of a solution containing paramidophenol 110 sulfate, an alkali sulfite, alkali carbonate, and an alkali hydrate in the proportion of 1/10 to 1/30 of the alkali carbonate.

3. A rapid, substantially stable photographic developing solution, consisting of a 115 solution in water of hydroquinone, paramidophenol sulfate, alkali sulfite, an alkali carbonate, and sodium hydrate in relatively small proportion to the alkali carbonate.

4. A rapid developing agent for sensitized 120 photographic surfaces, containing paramidophenol sulfate, a preservative, an alkali carbonate, and sodium hydrate in relatively small proportion to the alkali carbonate.

5. A rapid developing agent for sensitized 125 photographic surfaces, containing paramidophenol sulfate, an alkali carbonate, and an alkali hydrate in the proportion of 1/10 to 1/30 of the alkali carbonate.

6. A rapid, substantially stable, photo-

graphic developing solution, consisting of a solution in water of hydroquinone, 2 parts; paramidophenol sulfate, 1/2 part; sodium sulfite, 20 parts; sodium carbonate, 14 parts; 5 potassium bromid, 1/2 part; sodium hydrate, 1 part; all by weight, substantially as described.

7. A rapid, substantially stable, photographic developing solution, consisting of 10 a solution in water of hydroquinone, a paramidophenol salt, a preservative, an alkali carbonate, and sodium hydrate in relatively small proportion to the alkali carbonate.

8. A rapid developing agent for sensitized 15 photographic surfaces, containing paramidophenol sulfate, alkali carbonate, and an alkali hydrate in the proportion of 1/10 to 1/30 of the alkali carbonate.

9. A rapid, substantially stable, photographic developer, containing hydroquinone, paramidophenol sulfate, a preservative, an alkali carbonate, and sodium hydrate in rel-

atively small proportion to the alkali carbonate.

10. A rapid, substantially stable, photographic developer, containing hydroquinone, paramidophenol sulfate, a preservative, an alkali carbonate, and sodium hydrate in the proportion of 1/10 to 1/30 of the alkali carbonate. 25

11. A rapid, substantially stable, photographic developing solution, consisting of a solution in water of hydroquinone, paramidophenol sulfate, a preservative, a restrainer, an alkali carbonate, and sodium hydrate in 35 relatively small proportion to the alkali carbonate.

Signed at New York city in the county of New York and State of New York this 20th day of March A. D. 1915.

CHARLES J. THATCHER.

Witnesses:

ARTHUR WORSCHEK,  
LAURA E. SMITH.